

Feb. 23, 1971

J. W. FRONABARGER

3,565,932

LEAD HEXANITROOXANILIDE

Filed Feb. 12, 1969



Pb

INVENTOR  
JOHN W. FRONABARGER

BY

*Drummond, Cahill & Phillips*

ATTORNEYS

## 1

3,565,932

**LEAD HEXANITROOXANILIDE**  
John W. Fronabarger, Sun City, Ariz., assignor to UMC  
Industries, Inc., a corporation of Delaware  
Filed Feb. 12, 1969, Ser. No. 798,753  
Int. Cl. C07f 7/24  
U.S. Cl. 260—435

1 Claim

### ABSTRACT OF THE DISCLOSURE

A novel compound, lead hexanitrooxanilide, is a thermally stable, primary explosive exhibiting no-fire characteristics superior to those of lead styphnates.

This invention relates to explosives.

More particularly, the invention concerns a novel compound which is a thermally stable, primary explosive.

In a particular aspect, the invention concerns a thermally stable, primary explosive which exhibits no-fire characteristics superior to those of the lead styphnates.

In forming explosive trains, it is common practice to employ a so-called "primary" explosive which is thermally sensitive to initiation by thermal initiators such as bridgewires, pyrotechnics, and the like. The primary explosive should deflagrate or explode rather than burn, even when unconfined. Ordinarily, a primary explosive requires a relatively low energy input for its initiation, say on the order of 100,000 ergs or less.

By contrast, a "secondary" explosive requires a considerably higher energy input for initiation especially in the range of one billion ergs or greater and will not produce a high order detonation when burned unless suitably confined.

Lead styphnates are commonly employed in the explosive arts as primary explosives. However, it would be

## 2

highly desirable to provide a material of improved insensitivity to ignition from extraneous energy sources.

I have now discovered a novel compound which exhibits such characteristics and which is thermally stable, i.e., at 450° F. for at least two hours.

5 My novel compound is lead hexanitrooxanilide and has the structural formula shown in the drawings, according to present information.

My novel compound is lead hexanitrooxanilide and has the following method:

10 On hundred g. of 2,2',4,4',6,6'-hexanitrooxanilide is added to a warm (40° C.) stirred mixture of 3750 ml. of methanol and 1250 ml. of acetone. A warm solution of 100 g. of lead acetate trihydrate in 400 ml. methanol is

15 added to the resulting suspension with stirring. The resulting mixture is stirred for ten minutes subsequent to the lead acetate addition and the solid product is collected on a vacuum filter. After washing the product three times with 100 ml. portions of methanol and acetone, respectively, the solid is boiled in 200 ml. of methanol on a steam bath for five minutes. The purified solid is then collected on a vacuum filter, and washed three times with 100 ml. portions of methanol. Drying at 100° C. affords a product suitable for use.

20 25 Having described my invention and the presently preferred methods of practice thereof, I claim:  
1. Lead 2,2',4,4',6,6'-hexanitrooxanilide.

### References Cited

#### UNITED STATES PATENTS

2,150,653 3/1939 Franz et al. ----- 260—435

TOBIAS E. LEVOW, Primary Examiner

H. M. S. SNEED, Assistant Examiner

U.S. Cl. X.R.

149—105

UNITED STATES PATENT OFFICE  
CERTIFICATE OF CORRECTION

Patent No. 3,565,932

Dated February 23, 1971

Inventor(s) John W. Fronabarger

It is certified that error appears in the above-identified patent and that said Letters Patent are hereby corrected as shown below:

Column 1, line 30, "ralatively" should read -- relativel  
Column 2, line 5, "hurs" should read -- hours --; line 6,  
"hexanitrooanilide" should read -- hexanitrooxanilide --;  
lines 9 and 10, "My novel compound is lead hexanitrooxanili  
and has lowing method:" should read -- My novel compound is  
prepared according to the following method: --; line 20, "2  
should read -- 2000 --.

Signed and sealed this 12th day of September 1972.

(SEAL)

Attest:

EDWARD M. FLETCHER, JR.  
Attesting Officer

ROBERT GOTTSCHALK  
Commissioner of Patents